

Patented July 19, 1932

1,868,071

# UNITED STATES PATENT OFFICE

LEVI SCOTT PADDOCK, OF CHICAGO, ILLINOIS, ASSIGNOR TO SWIFT AND COMPANY, OF CHICAGO, ILLINOIS, A CORPORATION OF ILLINOIS

## MEAT STAMPING INK

No Drawing.

Application filed June 8, 1929. Serial No. 369,526.

This invention relates to meat marking inks suitable for use in rotary marking devices as distinguished from meat stamps which do not require a continuously operative ink feeding means.

The main objects of this invention are to provide an ink adapted to print on meat a brown impression which will simulate a burned brand, which will flow readily on a needle stamp, and which gives a clean-cut impression without smudge on a surface containing animal fats.

I have found that the proper color is obtained by using 9 parts of yellow A B and one part of methyl violet base. These animal line colors are soluble in fatty acids. It is well known that fatty acids are used as a solvent and vehicle when slow drying is essential as on ordinary rubber stamp pads and typewriter ribbons. Rubber stamp ink is a failure when the stamp is placed on meats where animal fats are present. The result is a spread of the ink into the fatty content since the fat is a solvent of the coloring matter used. Writing with ordinary water ink on moist paper is an example of the spread of the color into its own solvent.

I have found that it is necessary to abandon the use of oleic and similar acids as a vehicle, and have substituted ethyl alcohol containing about 10% ether. The result is a quick drying, sharp marking ink which will flow on a needle stamp.

A formula which I have found to be successful for carrying out the purpose of this invention is as follows:

9 grams yellow A B  
1 gram methyl violet base  
1 gram oleic acid  
900 C. C. ethyl alcohol  
100 C. C. ether

An illustrative procedure of the preparation of the ink by this formula is to take 1 gram methyl violet base, dissolve it in 1 gram oleic acid, add 9 grams of yellow A B and finally dissolve the dyes in 1,000 cubic centimeters of ethyl alcohol denatured with 10% ether; the oleic acid used being less

than 5% of the amount required to dissolve both colors.

I claim:

1. A brown ethyl alcohol ink consisting of yellow A B, methyl violet base, ether, 55 and sufficient oleic acid to partially dissolve the methyl violet.

2. A needle stamp ink adapted to simulate a burned-brand on meats using ethyl alcohol as a vehicle, yellow A B, and methyl 60 violet base for color, oleic acid to dissolve the methyl violet.

3. A brown color needle stamp ink consisting of 9 parts of yellow A B, 1 part methyl violet base, 1000 parts ethyl alcohol 65 containing 10% ether, and 1 part of oleic acid.

4. A rapid drying meat branding needle stamp ink containing nine parts of yellow A B, one part methyl violet base for one 70 thousand parts of alcohol containing 10% ether.

Signed at Chicago this 5th day of June, 1929.

LEVI SCOTT PADDOCK. 75

80

85

90

95

100